# NEW EUROPEAN PATENT SPECIFICATION

(11) **EP 0 717 161 B2**
(45) Date of publication and mention of the opposition decision: **27.03.2002**
(45) Mention of the grant of the patent: 25.11.1998
(21) Application number: 95850227.0
(22) Date of filing: 14.12.1995
(51) Int. Cl.: E04F 15/08, E04F 15/18, C04B 26/14

(54) **A tile floor and a process for production thereof**
Fliesenfussboden und sein Herstellungsverfahren
Plancher à carreaux et procédé pour sa réalisation

(30) Priority: 14.12.1994 SE 9404361
(43) Date of publication of application: 19.06.1996
(73) Proprietor: Akzo Nobel Decorative Coatings AB, 100 61 Stockholm (SE)
(72) Inventor: Hilgenbrink, Bernhard, 48565 Steinfurt-Borghorst (DE); Hermann, Günther, 48653 Coesfeld (DE)
(74) Representative: Fett, Günter

(56) References cited:
- DE-A- 2 348 301
- DE-A- 4 111 152
- US-A- 2 263 193
- PATENT ABSTRACTS OF JAPAN vol. 017, no. 577 (C-1122), 20 October 1993 & JP-A-05 170496 (DENKI KAGAKU KOGYO KK), 9 July 1993,
- Fachbuch:"Industriefußböden", P. Seidler,K. Beckmann, 1.Auflage, Grafenau/Württ., Lexika-Verlag,1978
- Fachbuch:"Bautenschutztaschenbuch", Schutz der Bauwerke vor Wässern und aggressiven Medien, Wolf-Peter Ettel, Hans-Dieter Wolf, Wolfram Diecke, 2.Auflage, Verlag für Bauwesen, 1992
- "Richtlinien zur Eingnunsfeststellung von Plattenbelägen" herausge geben von der Arbeitsgemeinschaft Industriebau e.V. (AGI), November 1991
- Arbeitsblatt S10,"Schutz von Baukonstruktionen mit Plattenbelägen gegen chemische Angriffe", Teil 1 bis 4, herausgegeben von der Arbeitsgemein- schaft Industriebau e.V., November 1991
- Fachbuch: "Industriefussböden", P. Seidler, K. Beckmann, 1.Auflage, Grafenau/Württ., Lexika-Verlag, 1978
- "Richtlinien zur Eignungsfeststellung von Plattenbelägen" herausgegeben von der Arbeitsgemeinschaft Industriebau e.V. (AGI), November 1991

## Description

This invention is related to a tile floor and a process for production thereof, especially a tile floor which is resistant to chemicals, such as acids, and is impervious to liquids, especially acids.

Tile floors are per se well-known for indoor as well as outdoor use, such as in industry buildings, and are often required to be resistant to chemicals and impervious to liquids, and are also often subjected to repeatedly applied high mechanical loads. For said purpose it is known to apply e.g. ceramic tiles on a base of mortar, optionally with a layer of a binding material, such as a cement slurry, and also to seal the layer of tiles with a sealing material applied in the gaps between adjacent tiles. The top layer of tiles is sometimes subjected to a vibration treatment with vibrating tools for consolidating or compacting the underlying layer and improving the contact with the tile layer.

As examples of such prior art processes reference can be made to DE 23 48 301, DE 25 45 925, DE 27 54800, DE 41 11 152 A1 and EP 0 340 598 A2, which disclose tile floors in which the gaps between the tiles are filled with acid resistant materials These and other processes and the products thereof have, however, until now exhibited several disadvantages. Among these disadvantages is that such previously known tile floors are difficult, time consuming and expensive to produce and/or are vulnerable to the formation of cracks caused by high stresses and impact loads which are not uncommon for tile floors, especially for tile floors in e.g. industry buildings. Such cracks are particularly objectionable when the floor should also be resistant and impervious to chemicals, especially liquids.

The present invention makes it possible to achieve one or more of the following advantages in relation to the prior art: improved resistance against chemicals, improved imperviousness and/or crack resistance of the tile floor, also when subjected to high stresses and high impact loads, reduction of the time required for laying the floor, reduction of the time required until the floor can support loads, simplified laying of the floor, reduced risk of undesired intermixing of floor layers, improved bonding of the floor layers, reduced consumption of floor materials, such as bonding materials, especially organic binders, etc. and/or reduced material and labour costs.

The floor tiles used for the tile floor according to this invention can be of various types which have also previously been used as an upper or top layer of floors, such as tiles made from metallic materials, natural or artificial stone, wood products, concrete, plastics and especially ceramics, e.g. glazed or unglazed ceramics, such as dry-pressed and sintered ceramic floor tiles.

The present invention is defined by the claims.

The upper surface of the structural member and/or the base layer should suitably have a shape, e.g. a slope, which fairly closely coincides with the desired shape of the tile layer forming the top of the floor, e.g. a distance in the vertical direction between the base layer and the upper surface of the tile layer which within the main part of the surface area of the floor deviates less than 20 cm and preferably approximately 5 cm from the average value of said distance within said surface area, and/or an average deviation of angle of slope within said area of less than 10 and preferably less than 3 degrees. Usually the angle of slope of the tile layer is more than zero degrees from the horizontal. A suitable degree of flatness is defined in DIN 18 202.

A suitable material for said base layer is concrete or mortar, especially cement mortar, and the base layer may comprise reinforcements, such as embedded reinforcements, e.g. steel rods and steel mesh reinforcements. The material, from which the base layer is made, comprises usually a mixture of a binder phase, especially an inorganic hydraulic binder, such as cement, e.g. Portland cement or aluminous cement, and particulate fillers or aggregates, especially sand, gravel and similar materials. An example of a suitable filler is sand, preferably washed sand, with a grain size (grading curve) within the range 0 to 8 mm. As is well-known in the art also coarser aggregate fractions may be present in the mix, such as crushed aggregates for concrete, gravel, cobbles, puddingstones, expanded clay, etc. The mixing ratio of binder, especially cement, e.g. Portland cement, to filler, especially sand, is often suitably at least 1:2 or at least 1:4, and optionally up to 1:10 or up to 1:8, e.g. about 1:6. A suitable water/cement ratio is e.g. about 0.5, but also higher or lower values can be used, e.g. up to 0,8 and down to 0,3.

The cured strength of the base layer mortar could suitably at least correspond to ZE 12 according to DIN 18 560. This corresponds usually to a cement content of at least 240 kg of cement per cubic metre of fresh cement mortar.

An intermediate layer is suitably applied on the base layer. The purpose of the intermediate layer is especially to prevent, completely or at least partially, mixing of the base layer material into the bonding layer used for bonding the tiles, and especially to reduce penetration of the bonding material into the base material layer to a comparatively narrow zone at the interface of the bonding material/base layers, and/or to permit convenient application of the bonding layer material on to the base layer. The intermediate layer is important especially in case the bonding layer material is applied on to an incompletely cured (set) or substantially uncured base material, and/or a base material still showing plasticity or consistency, such as earth-moist, fluid, harsh, plastic or semi-fluid consistency, e.g. as measured with various well-known measuring devices, such as Mo, flow table, slump cone, Thaulow, vebe and other measuring devices, and/or on an incompletely compacted or uncompacted base layer, in which case it may be difficult to apply the bonding material as a layer, such as an even layer or as a layer of strings, e.g. with a trowel (teeth-trowel), and/or the bonding material and the base layer material may, or have a tendency to, intermix excessively, in which case a substantial part of the bonding material may become lost in the base layer and unable to bind to the tiles.

Preferably the bonding material forms an interface with the base material layer at or below the lower surface of the intermediate material layer, preferably over at least 40%, at least 60% or at least 80% or substantially 100% of the areal extension of the base material surface below the intermediate/bonding material layers. A certain degree of penetration of the bonding material into the base material can help to improve the bonding to the base material layer, e. g. penetration to an average depth of at least 1 mm, at least 3 mm or at least 5 mm, and optionally up to at most 20 mm, at most 10 mm or at most 6 mm into the base material layer.

The intermediate layer should preferably be at least partially permeable to the bonding material used in the bonding layer, e.g. comprise perforations, open pores or openings, e.g. between fibres or fibre yarns, which permit penetration thereof by the bonding material. This porosity includes the porosity present in a fibre material, especially textile fibre material. Such fibrous materials may have an average fibre diameter of e.g. at least 0,01, at least 0,05 mm or at least 0,1 mm and optionally up to at most 2 mm, at most 1mm or at most 0,1 mm. The porosity may comprise an average pore size of from at least 0,01 mm, at least 0,1 mm or at least 1 mm and optionally up to at most 5 mm or at most 1 mm, depending upon the type of porous material. The porous intermediate material is preferably flexible, so that it by its own weight, and optionally when loaded with the bonding material, tightly follows the shape of the base material layer on which it is laid, e.g. with a distance between the intermediate material layer and the substrate, such as the base layer, calculated as an average over the areal extension of the intermediate layer, of at most 10 mm or at most 1 mm. The flexibility may be such that the intermediate material without difficulty can be winded up on a roll (e.g. a roll with a diameter of at most 25 times the thickness of the intermediate material). The intermediate layer material may consist e.g. of such fibrous materials as woven or non-woven or other textile materials. Suitable materials for the intermediate layer are thus e.g. fleece materials, this expression being taken in a broad meaning, e.g. non-woven materials, felted materials, woven materials, fabrics, stitched, knitted or hoistery products, of organic and/or inorganic materials, such as glass, stone, organic polymers, such as polyamides, polyesters, polyolefines, e.g. polyethylene, polypropylene, acrylic polymers, vinylic polymers, etc., preferably mainly in the shape of fibres or products made from fibres, e.g. glass fibre materials, polyamide fibre materials, polyester fiber materials, other textiles, or porous products. Suitable are e.g. materials of the lightweight non-woven type, e.g. based on one or more of the materials mentioned above, e.g. polyester, polyamide, polypropylene, polyethylene, glass fibres and natural fibres. Suitable are usually materials of the geotextile type and other materials which are commonly used as intermediate layers, e.g. between different materials, such as materials of different grain size ranges, e.g. in road construction, building industry etc.

The intermediate layer should preferably have characteristics which make it possible to lay down a layer of the material on the base layer, especially before partial or complete curing or setting of such a base layer, and/or make it possible to subject the intermediate material layer to a certain amount of mechanical interaction, e.g. by applying a layer of liquid or flowable bonding material thereon, preferably as a layer of even thickness, optionally with or in the form of strings, e.g. with trowels, such as trowels with or without teeth, or other means, without the formation of wrinkles or other irregularities in the intermediate material layer or without removal of said layer from the underlying surface. The intermediate material may be supplied as a web material, which can be laid down as pieces of suitable length and width, e.g. as overlapping pieces, on the base layer or supporting member. Preferably the pieces are laid down in parallel and/or crossing directions. One or more such layers of intermediate material, especially web, may be applied on the substrate. The weight per square metre of the intermediate layer may amount to e.g. at least 10, at least 20 or at least 50 grams, and a suitable upper limit of the weight may be up to 500 or up to 300 grams, e.g. a fleece (non-woven) with a weight of 30 to 240 grams per square metre, and suitably a tensile strength according to DIN 53857-2 of at least 1 or at least 3 KN and up to e.g. 15 or up to 8 KN. The thickness of a web or sheet material used in the intermediate material layer may be e.g. at least 0,1 mm, at least 0,5 mm or at least 1 mm, and optionally e.g. at most 10 mm, at most 5 mm, at most 2 mm or at most 1 mm. the intermediate material layer may be formed from one such web or sheet part or from 2 or more such parts arranged in a stack on each other. The porosity of the intermediate layer material, prior to impregnation with the bonding material, may amount to e.g. at least 60 %, and optionally e.g. at most 80 % or at most 60 %, preferably mainly as open, communicating porosity, depending e.g. upon the type of material. Examples of suitable materials are those produced and sold by Du Point Company under the trade mark "Typar", e.g. Typar 3207, 3267, 3337, 3407-2, 3707 and especially 3407, 3607-3 and 3857. These materials are disclosed e.g. in an information sheet from the producer with the title "Technische Daten Typar" (copy enclosed as Table 1). Similar products from other producers can also be used, preferably products with characteristics within. or essentially within, the ranges defined by the above mentioned "Typar" products, especially the upper and lower values for the various characteristics given for said products, particularly the especially mentioned three products.

The intermediate layer material is permeable to the bonding layer material so that a layer of the bonding material applied on the intermediate material will or can be brought to penetrate through the intermediate material layer to the surface, on which the intermediate material layer rests, i.e. usually the surface of the base layer or the structural member, and to form a bond to said surface. Furthermore, the material of the intermediate layer should preferably also permit impregnation of the intermediate layer with the bonding material, preferably so that open empty spaces or voids in the intermediate layer are filled, e.g. to at least 20 %, at least 50 %, at least 75 % or essentially completely filled with the bonding material in the finished tile floor. Optionally the intermediate material may also be impregnated with bonding material, e.g. to a percentage within the limits mentioned above, prior to applying the intermediate material on the substrate, especially the base material.

As indicated above, the bonding layer suitably comprises a bonding material which can bind to the floor tiles as well as to the intermediate layer and the base layer or the structural member in case no base layer is used. The bonding material may be of inorganic as well as organic origin, such as hydraulic binders, e.g. cement, such as Portland cement and aluminate cement, especially acid resistant cement, water glass, but preferably organic and especially polymeric binders (adhesives, glues etc.) are used, either alone or in combination, optionally with hydraulic binders; such as epoxy resins, polyurethanes, polyesters etc., e.g. as dispersions, such as aqueous dispersions and emulsions, especially of the two-component type. Examples of such two-component binders or two-component reactive resins are combinations of a resin component and a hardener component, in which the resin component may consist of a Bisphenol resin, such as Bisphenol A resin, Bisphenol F resin or Bisphenol A/F resin, e.g. with reactive diluents, such as a Glycidyl ether. The hardener may preferably consist of a "cold hardener", especially amine hardener, such as aliphatic polyamine, cycloaliphatic amine, aliphatic amine or aromatic amine hardener, e.g. modified amine hardener. The hardener, such as amine hardener, may suitably be of the type which can be emulsified in water. Also combinations of two or more such binders may be used. The bonding material is preferably combined with fillers, such as particulate or fibrous fillers, especially inert fillers, such as silica, e.g. silica flour, fire-clay, organic resin flour, organic resin granules etc. The particle size distribution of the fillers should preferably be selected so that the bonding material can penetrate through the intermediate material layer and also rise in the gaps between the tiles, e.g. when subjecting the tiles to a vibration treatment for compacting and consolidating the tile layer and optionally other parts of the floor below the tile layer.

When applying the bonding and/or intermediate layers on a fresh or non-cured base layer of mortar (e.g. cement mortar) which is damp, moist or still wet, the bonding material should preferably be resistant against wet and/or alkaline conditions and may preferably consist of water dispersible epoxy resin, acid resistant cements, dispersions, water glass or combinations of two or more such materials.

The bonding material should be resistant against and/or impervious to the materials against which the tile floor should be resistant and/or impervious. A number of such chemicals are mentioned in a pamphlet from Applicant with the title: "Schönox Fliesentechnik, Beständigkeitsliste, SCHÖNOPOX CON, SCHÖNOPOX CF". The bonding material is preferably resistant and impervious to one or more of the chemicals enumerated in the list in said pamphlet, especially to those marked with "+" or "(+)" in said list. Among such chemicals, in various concentrations, can be mentioned: organic acids, e.g. formic, acetic, lactic, oxalic, tartaric and citric acids, inorganic acids, e.g. boric, chromic, chloric, phophoric, nitric, hydrochloric and sulphuric acids, bases, e.g. ammonium, potassium and sodium hydroxides and carbonates, alkoholes, e.g. ethanol, isopropanol, butanol and phenols, hydrocarbons, e.g. petroleum, gasoline, kerosene, motor oil, turpentine, etc.

The tiles are suitably laid down with small gap widths between adjacent tiles, such as in average up to 15 mm, up to 10 mm, up to 5 mm, up to 2 mm or up to 1 mm, and usually at least 0,1 mm gap width. The gaps are preferably filled partly or completely with bonding material rising from the bonding layer, especially as a result of a compacting and consolidating treatment, especially mechanical, preferably vibration treatment, but can also be filled partly or completely with a bonding and/or sealing material, e.g. the material used in the bonding layer, supplied from the upper side of the tile layer. The tiles are preferably cleaned from any excess of bonding and/or sealing material at the gaps or on the upper surface of the tiles as soon as possible.

Devices and methods for consolidating or compacting tile floors are well-known. Vibrating devices can according to this invention be used with advantage for laying tile floors, and such devices and methods which are previously known to those skilled in the art can generally be used also for laying tile floors according to this invention. Examples of such devices are those produced by Firma Karl Dahm, Germany, such as those devices which are commercially availalble under the trade names "Doberman", "Alano", "Rüttelgerät KD I", "Rüttelgerät KD II" and "Handrüttelgerät KD II", and devices of similar types from other producers.

An embodiment of this invention is explained in the following example with reference to the enlosed drawing. This example is intended to illustrate the invention without in any way restricting the scope of the invention.

### Example

The enclosed drawing is a vertical cross section through a part of a tile floor according to this invention. The tile floor rests on a structural member for the tile floor consisting of a construction (not shown on the drawing) of concrete made from Portland cement and conventional aggregate. A base layer 1 of Portland cement mortar based on a mixture of 1 part of Portland cement and 6 parts of washed sand with a grading curve of 0 to 8 mm, and a quantity of coarser aggregate stones and with a water/cement ratio of 0.5, was applied on a welded steel rod reinforcement (not shown) to a layer thickness of about 10 cm, and screeded to make the surface smooth. The fresh, unhardened base layer was coated with an intermediate layer 2 of soft, synthetic polymer non-woven (fleece) of the geo-textile type with a surface weight of about 100 grams per square metre, a thickness of below 0,9 mm and a pore size range of mainly 0,1 to 1,5 mm, Said non-woven was delivered as web on rolls, which were available with a web width of 1 to 4 metres and a web length of 50 to 200 metres. Epoxy mortar based on epoxy resin of the water emulsifiable type (SCHÖNOPOX CON, SCHÖNOPOX CF, registered trade marks) containing silica flour as an inert filler was used as bonding material. The binding compound was a two-component water emulsifiable epoxy resin mortar, and the bonding material was applied on the intermediate layer with a trowels (with and without teeth) in a quantity which was sufficient for completely filling the voids in the intermediate layer, and for penetrating down through the intermediate layer into contact with the base layer and forming a continuous layer 3 on top of the intermediate layer. The epoxy mortar, which in the finished tile floor was penetrated through the intermediate layer 2, formed a penetration layer 4 at the interface of the intermediate layer 2 with the cement mortar base layer 1 with excellent bonding to the base layer On the bonding epoxy mortar layer 3 dry-pressed ceramic floor tiles 5 according to DIN EN 176 and DIN 18 158 were laid tightly abutting with a gap width of in average below 1 millimetre as a top layer. The tile floor layer was subjected to a vibration treatment with a vibrator of the type commonly used for vibrating tile floors. The vibration treatment was performed until it was decided that the base layer and the bonding and intermediate layers were consolidated and compacted with removal of voids from said layers and from the interfaces between the bonding layer and the bottom surfaces of the tiles, and penetration of the bonding material to the surface of the base layer was sufficient. By said vibration treatment the bonding material was brought to rise in the gaps 6 between the tiles, optionally essentially to the level of their upper surface, or to a lower level, in which case the gaps were filled from above with a grout consisting essentially of the same material as the epoxy mortar used for the bonding layer 3. The surface of the tile layer was then cleaned from any bonding material which had been spread onto the tile surfaces. The finished floor was resistant to acids and impervious to liquids and exhibited high mechanical strength, with the intermediate non-woven layer 2 acting as a reinforcement of the bonding epoxy mortar layer 3, and also as a barrier against penetration of the concrete material of the base layer up into the epoxy mortar layer 3.

Alternative embodiments of the invention are obvious to those skilled in the art from the disclosure above.

**Table 1**

| Properties | Test method | Unit | 3207 | 3267 | 3337 | 3407 | 3407-2 | 3607-3 | 3707 | 3857 |
|---|---|---|---|---|---|---|---|---|---|---|
| Mechanical properties | | | 0,70 | 0,75 | | | | | | |
| | | | | | | | | | | |
| Punch push - through force (x) | DIN 54307 | N | 500 | 690 | 830 | 1270 | 1500 | 1850 | 2450 | 3030 |
| | | | | | | | | | | |
| Class value (x-s) | | | - | - | 609 | 1152 | 1350 | 1784 | 2250 | 2904 |
| | | | | | | | | | | |
| Fleeche class | | | 1 | 1 | 1 | 2 | 2 | 3 | 3 | 4 |
| | | | | | | | | | | |
| Tear strength from | DIN 53857-2 | kN/m | 3,1 | 4,1 | 5,0 | 7,6 | 8,8 | 10,3 | 14,2 | 17,4 |
| stripe tensile | | N/10 cm | 310 | 410 | 500 | 760 | 880 | 1030 | 1420 | 1740 |
| test | | N/ 5 cm | 155 | 205 | 250 | 380 | 440 | 515 | 710 | 870 |
| | | | | | | | | | | |
| Elongation at break from stripe tensile test | DIN 53857-2 | % | 35 | 40 | 40 | 40 | 40 | 40 | 40 | 40 |
| Grab tensile test | DIN 53858 | N | 270 | 360 | 440 | 565 | 710 | 890 | 1070 | 1300 |
| | | | | | | | | | | |
| Elongation at break from grab tensile test | | % | >60% | >60% | >60% | >60% | >60% | >60% | >60% | >60% |
| Area weight | DIN 53854 | 9/m² | 68 | 90 | 110 | 136 | 150 | 190 | 240 | 290 |
| | | | | | | | | | | |
| Thickness | DIN 53855/3 | mm | | | | | | | | |
| at 2 kN/m² load | | | 0,36 | 0,41 | 0,45 | 0,46 | 0,48 | 0,56 | 0,68 | 0,78 |
| at 20 kN/m² load | | | 0,33 | 0,36 | 0,40 | 0,43 | 0,44 | 0,52 | 0,65 | 0,75 |
| at 200 kN/m² load | | | 0,29 | 0,34 | 0,35 | 0,39 | 0,40 | 0,48 | 0,63 | 0,72 |
| Hydraulic properties | | | | | | | | | | |
| | | | | | | | | | | |
| Flow rate Q at 10 cm water head | DE VOORST | 1/m² x s | 260 | 210 | 160 | 100 | 75 | 60 | 40 | 30 |
| | | | | | | | | | | |
| "Water permeability" k under 2 kN/m² load | EMPA/ITF/Franzlus | *m/s (x 10⁻⁴) | 25 | 13 | 10 | 7 | 5 | 6,5 | 4,0 | 3,5 |
| | | m/s | 0,0025 | 0,0013 | 0,001 | 0,0007 | 0,0005 | 0,00065 | 0,0004 | 0,00035 |
| | | cm/s | 0,25 | 0,13 | 0,1 | 0,07 | 0,05 | 0,065 | 0,04 | 0,035 |
| | | | | | | | | | | |
| "Water permeability" k under 200 kN/m² load | EMPA/ITF/ Franzlus | *m/s (x10⁻⁴) | 9 | 7 | 6 | 5 | 3,5 | 5 | 2,8 | 2,1 |
| | | m/s | 0,0009 | 0,0007 | 0,0006 | 0,0005 | 0,00035 | 0,0005 | 0,00028 | 0,00021 |
| | | cm/s | 0,09 | 0,07 | 0,06 | 0,05 | 0,035 | 0,05 | 0,025 | 0,021 |
| | | | | | | | | | | |
| Effective opening diameter | Franzlus/EMPA | mm | 0,27 | 0,25 | 0,19 | 0,14 | 0,13 | 0,1 | 0,09 | 0,07 |
| D_{W(90)} | | micron | 270 | 250 | 190 | 140 | 130 | 100 | 90 | 70 |

| | | | | | | | | | | |
|---|---|---|---|---|---|---|---|---|---|---|
| *also m/s E-4 The stated values are within the testing accuracy of the laboratory test in question. Changes may occur. ^{x}Du Pont's registered Trade Mark | | | | | | | | | | |

## Claims

1. A process for laying a tile floor which is resistant to chemicals and impervious to liquids, the process comprising the following steps:
• applying a base layer (1) on a supporting structural member;
• applying at least one layer (3) of bonding material suitable for forming a chemical resistant and liquid impermeable continuous layer;
• laying a layer of floor tiles (5) on the layer of bonding material;
• consolidating and compacting the floor by subjecting the floor tile layer to a mechanical compacting treatment, thereby forming a tight bonding contact between the floor tiles (5) and the underlying continuous bonding material layer (3)
**characterized in that** an intermediate layer (2) of fibre material is applied onto the base layer (1) when the base layer is still at most in completely set substantially and especially fresh and unhardened, the intermediate layer (2) being permeable to the bonding material but substantially impermeable to the material of the base layer, the bonding material penetrating through the intermediate layer within at least a part of the areal extension of the intermediate layer, thereby at least contributing to the bonding of the floor tile layer and the intermediate layer to the base layer (1).

2. A process according to claim 1 **characterized in that** the fibre material used for the intermediate layer has a weight per m² of 10 - 500 grams, preferably of 20 - 300 grams, the fibres having a diameter of 0,01 - 2 mm, preferably about 0,1 mm.

3. A process according to either of the preceding claims, **characterized in that** the compacting treatment is a vibrating treatment.

4. A mechanically compacted and consolidated tile floor which is resistant to chemicals and impervious to liquids, said floor comprising a top layer of floor tiles (5), a substrate for said floor tile layer comprising a supporting structural member, and a bonding material layer (3) comprising bonding material which binds the floor tile layer to the substrate, the substrate comprising a base material layer (1), the tile floor having been compacted by mechanical compacting treatment, **characterized in that** the substrate also comprises a mainly fibre based intermediate material layer (2), applied as at least one layer (2) on to an at most incompletely set and especially fresh, unhardened base material layer of the substrate, on to which the floor tile layer is bonded with the bonding material, the bonding material penetrating through the mainly fibre based intermediate material layer and bonding to said base material layer within at least a part of the areal extension of the intermediate material layer, thereby at least contributing to the bonding of the floor tile layer and the intermediate material layer to the underlaying substrate, the tile floor being substantially free from penetration of the base material layer, upon which the intermediate material layer rests, into the bonding material layer (3) above the intermediate material layer (2), or at most exhibits penetration of material from the base material layer into the intermediate material layer up to at most a part of the thickness of the intermediate material layer.

5. A tile floor laid according to claim 4, **characterized in that** the tiles are laid with gaps between them having a width of less than 2 mm.

6. A tile floor according to claim 5, **characterized in that** the gaps between the tiles have a width of less than 1 mm, preferably less than 0,1 mm.

7. A tile floor according to claim 5 or 6, **characterized in that** the tiles are tightly abutting.

8. A tile floor according to claim 4-7, **characterized in that** the intermediate layer comprises a geo-textile type of fibre material.

9. A tile floor according to any one of the preceding claims 4, 5, 6, 7, or 8, **characterized in that** the floor comprises as a base layer, under the intermediate layer, a mortar layer consisting of a combination of aggregates and mortar binder selected from the group consisting of hydraulic cements, gypsum and organic resins.

## Patentansprüche

1. Verfahren zum Legen eines Fliesenbodens, der chemikalienbeständig und flüssigkeitsundurchlässig ist, wobei das Verfahren die folgenden Schritte umfasst:
- Auftragen einer Grundschicht (1) auf ein tragendes Strukturelement;
- Auftragen wenigstens einer Schicht (3) eines Klebematerials, das zur Bildung einer chemikalienbeständigen und flüssigkeitsundurchlässigen kontinuierlichen Schicht geeignet ist;
- Legen einer Schicht von Bodenfliesen (5) auf die Schicht aus Klebematerial;
- Verfestigen und Kompaktieren des Bodens, indem man die Bodenfliesenschicht einer mechanischen Kompaktierungsbehandlung unterzieht, wodurch ein dichter Klebekontakt zwischen den Bodenfliesen (5) und der darunterliegenden kontinuierlichen Schicht aus Klebematerial (3) entsteht;
**dadurch gekennzeichnet, dass** eine Zwischenschicht (2) aus Fasermaterial auf die Grundschicht (1) aufgetragen wird, wenn die Grundschicht höchstens noch unvollständig gehärtet und insbesondere noch frisch und ungehärtet ist, wobei die Zwischenschicht (2) für das Klebematerial durchlässig ist, aber für das Material der Grundschicht im wesentlichen undurchlässig ist, wobei das Klebematerial wenigstens innerhalb eines Teils der Flächenerstreckung der Zwischenschicht durch die Zwischenschicht dringt, wodurch es zum Kleben der Bodenfliesenschicht und der Zwischenschicht auf der Grundschicht (1) wenigstens beiträgt.

2. Verfahren gemäß Anspruch 1, **dadurch gekennzeichnet, dass** das für die Zwischenschicht verwendete Fasermaterial ein Gewicht pro m² von 10 bis 500 Gramm, vorzugsweise 20 bis 300 Gramm, hat, wobei die Fasern einen Durchmesser von 0,01 bis 1 mm, vorzugsweise etwa 0,1 mm, haben.

3. Verfahren gemäß einem der vorstehenden Ansprüche, **dadurch gekennzeichnet, dass** die Kompaktierungsbehandlung eine Vibrationsbehandlung ist.

4. Mechanisch kompaktierter und verfestigter Fliesenboden, der chemikalienbeständig und flüssigkeitsundurchlässig ist, wobei der Boden eine Deckschicht aus Bodenfliesen (5), ein Substrat für die Bodenfliesenschicht mit einem tragenden Strukturelement sowie eine Schicht aus einem Klebematerial (3) mit Klebematerial, das die Bodenfliesenschicht mit dem Substrat verklebt, umfasst, wobei das Substrat eine Grundmaterialschicht (1) umfasst, wobei der Fliesenboden durch mechanische Kompaktierungsbehandlung kompaktiert worden ist, **dadurch gekennzeichnet, dass** das Substrat auch eine hauptsächlich auf Fasern beruhende Zwischenmaterialschicht (2) umfasst, die als wenigstens eine Schicht (2) auf die höchstens noch unvollständig gehärtete und insbesondere noch frische und ungehärtete Grundmaterialschicht des Substrats aufgetragen ist, auf das die Bodenfliesenschicht mit dem Klebematerial geklebt wird, wobei das Klebematerial wenigstens innerhalb eines Teils der Flächenerstreckung der Zwischenmaterialschicht durch die hauptsächlich auf Fasern beruhende Zwischenmaterialschicht dringt und an der Grundmaterialschicht klebt, wodurch es zum Kleben der Bodenfliesenschicht und der Zwischenmaterialschicht auf dem darunterliegenden Substrat wenigstens beiträgt, wobei der Fliesenboden im wesentlichen frei von Durchdringen der Grundmaterialschicht, auf der die Zwischenmaterialschicht ruht, in die Klebematerialschicht (3) oberhalb der Zwischenmaterialschicht (2) ist oder höchstens ein Durchdringen von Material aus der Grundmaterialschicht in die Zwischenmaterialschicht bis zu höchstens einem Teil der Dicke der Zwischenmaterialschicht aufweist.

5. Fliesenboden, der gemäß Anspruch 4 gelegt wurde, **dadurch gekennzeichnet, dass** die Fliesen mit dazwischen befindlichen Lücken mit einer Breite von weniger als 2 mm gelegt werden.

6. Fliesenboden gemäß Anspruch 5, **dadurch gekennzeichnet, dass** die Lücken zwischen den Fliesen eine Breite von weniger als 1 mm, vorzugsweise weniger als 0,1 mm, haben.

7. Fliesenboden gemäß Anspruch 5 oder 6, **dadurch gekennzeichnet, dass** die Fliesen dicht aneinanderstoßen.

8. Fliesenboden gemäß Anspruch 4 bis 7, **dadurch gekennzeichnet, dass** die Zwischenschicht ein Fasermaterial des Geotextiltyps umfasst.

9. Fliesenboden gemäß einem der vorstehenden Ansprüche 4, 5, 6, 7 oder 8, **dadurch gekennzeichnet, dass** der Boden als Grundschicht unter der Zwischenschicht eine Mörtelschicht umfasst, die aus einer Kombination von Zuschlägen und Mörtelbindemitteln, die aus der aus hydraulischen Zementen, Gips und organischen Harzen bestehenden Gruppe ausgewählt sind, besteht.

## Revendications

1. Procédé pour poser un carrelage, qui est résistant aux produits chimiques et imperméable aux liquides, le procédé comprenant les étapes consistant à :
- appliquer un couche de base (1) sur un élément de structure ;
- appliquer au moins une couche (3) de matière liante appropriée pour former une couche continue résistant aux produits chimiques et imperméable aux liquides ;
- poser une couche de carreaux (5) sur la couche de matière liante ;
- consolider et compacter le sol en soumettant la couche de sol carrelé à un traitement de compactage mécanique, pour former une liaison de contact ferme entre les carreaux de sol (5) et la couche continue de matière liante sous-jacente (3) ;
**caractérisé en ce qu'**une couche intermédiaire (2) de matériau fibreux est appliquée sur la couche de base (1) quand la couche de base est encore au moins incomplètement prise et en particulier, fraîche et non durcie, la couche intermédiaire (2) étant perméable à la matière liante mais sensiblement imperméable au matériau de la couche de base, la matière liante pénétrant au travers de la couche intermédiaire sur au moins une partie de l'étendue de la couche intermédiaire, contribuant ainsi au moins en partie, à la liaison de la couche de carreaux et de la couche intermédiaire à la couche de base (1).

2. Procédé selon la revendication 1, **caractérisé en ce que** le matériau fibreux utilisé pour la couche intermédiaire a un poids par mètre carré allant de 10 - 500 g, de préférence de 20 - 300 g, les fibres ayant un diamètre allant de 0,01 - 2 mm, de préférence d'environ 0,1 mm.

3. Procédé selon l'une quelconque des revendications précédentes, **caractérisé en ce que** le traitement de compactage est un traitement par vibration.

4. Sol carrelé compacté et consolidé de façon mécanique, qui est résistant aux produits chimiques et imperméable aux liquides, ledit sol comprenant une couche supérieure de carreaux (5), un substrat pour ladite couche de carreaux, comprenant un élément de structure et de support, et une couche de matière liante (3) comprenant une matière liante qui lie la couche de carreaux au substrat, le substrat comprenant une couche de matériau de base (1), le carrelage ayant été compacté par un traitement de compactage mécanique, **caractérisé en ce que** le substrat comprend également une couche de matériau intermédiaire principalement à base de fibres (2), appliquée sous la forme d'au moins une couche (2) sur une couche du matériau de base au moins incomplètement pris et en particulier, frais, non durci, du substrat sur lequel la couche de carreaux est liée avec la matière liante, celle-ci pénétrant au travers de la couche de matériau intermédiaire à base surtout de fibres et la liant à la dite couche de matériau de base sur au moins une partie de l'étendue de la couche de matériau intermédiaire, en contribuant ainsi, au moins en partie, à la liaison de la couche de carreaux et de la couche de matériau intermédiaire au substrat sous-jacent, le sol carrelé étant sensiblement exempt de pénétration du matériau de base, sur lequel la couche de matériau intermédiaire repose, dans la couche de matière liante (3) par dessus la couche de matériau intermédiaire (2), ou au plus montre une pénétration de matière de la couche de matériau de base dans la couche de matériau intermédiaire jusqu'au plus une partie de l'épaisseur de la couche de matériau intermédiaire.

5. Sol carrelé posé selon la revendication 4, **caractérisé en ce que** les carreaux sont posés avec des intervalles entre eux d'une largeur inférieure à 2 mm.

6. Sol carrelé selon la revendication 5, **caractérisé en ce que** les intervalles entre les carreaux ont une largeur inférieure à 1 mm, de préférence inférieure à 0,1 mm.

7. Sol carrelé selon la revendication 5 ou 6, **caractérisé en ce que** les carreaux sont assemblés en about.

8. Sol carrelé selon les revendications 4 à 7, **caractérisé en ce que** la couche intermédiaire comprend un matériau fibreux de type géotextile.

9. Sol carrelé selon l'une quelconque des revendications précédentes 4, 5, 6, 7 ou 8, **caractérisé en ce que** le sol comprend comme une couche de base, en dessous de la couche intermédiaire, une couche de mortier consistant en une combinaison d'agrégats et de mortier liant sélectionné parmi un groupe consistant en les ciments hydrauliques, le plâtre et les résines organiques.
